

Feb. 5, 1924.

1,482,789

E. C. GMELIN

METHOD OF MAKING GLASS LETTERS

Filed March 30, 1921

3 Sheets-Sheet 1

Fig. 1.



Fig. 2.



Fig. 3.



Witness:  
Stephen M. Morris

Fig. 4.



Inventor:  
Eugene C. Gmelin,

By Dyrenforth, Lee, Chittenden & Wilcox, Attys.

Feb. 5, 1924.

1,482,789

E. C. GMELIN

METHOD OF MAKING GLASS LETTERS

Filed March 30, 1923

3 Sheets-Sheet 2

Fig. 5.



Fig. 6.



Fig. 9.



Fig. 8.



Witness:

Stephen Hebra

Inventor:

Eugenio C. Gmelin,

Duvenborth, Chuttle & Wiles, Attorneys

Feb. 5, 1924.

1,482,789

E. C. GMELIN

METHOD OF MAKING GLASS LETTERS

Filed March 30, 1921

3 Sheets-Sheet 3



Witness:

*Stephen Kibria*

Inventor:  
Eugene C. Gmelin.

*As Dyenforth, Lee, Chitten & Wiles, Attns.*

Patented Feb. 5, 1924.

1,482,789

# UNITED STATES PATENT OFFICE.

EUGENE C. GMELIN, OF CHICAGO, ILLINOIS.

## METHOD OF MAKING GLASS LETTERS.

Application filed March 30, 1921. Serial No. 457,158.

To all whom it may concern:

Be it known that I, EUGENE C. GMELIN, a citizen of the United States, residing at 407 North Wells Street, Chicago, in the county of Cook and State of Illinois, have invented a new and useful Improvement in Methods of Making Glass Letters, of which the following is a specification.

This invention relates to improvements in the method of forming raised glass letters or other characters in sheets of glass. For convenience of description I have shown the method of forming the letter "E"; although it is obvious that, without detracting from the spirit of this invention, any other letter, or any numeral, or character, or figure of any kind could be formed by use of my invention.

One method, embodying the features of my invention, of forming a letter, is disclosed in the accompanying drawings in which Figure 1 is a view in elevation of a blow-torch used in the practice of my invention, Fig. 2 is a vertical sectional view of the atomizing-nozzle forming a part of the blow-torch, Fig. 3 is a vertical sectional view of a burner-tip of the blow-torch, Fig. 4 is a view taken as indicated by line 4 of Fig. 3, Fig. 5 is a perspective view showing a die in place on a table, to be used in connection with the form of a letter, Fig. 6 is a vertical sectional view of the die taken as indicated by line 6 of Fig. 5, Fig. 7 is a view in perspective of a sheet of glass from which a letter is to be formed, Fig. 8 is a view in perspective of a sheet of glass on the die after the letter has been formed, Fig. 9 is a view in perspective of the sheet of glass removed from the die and turned over showing the completed letter raised from the surface, Fig. 10 is a view in perspective of a step in the method of forming a letter, showing a letter partly formed.

As shown in the drawings A indicates in general a blow-torch adapted to be operated in the usual manner with gas and air. The torch includes a T connection 10 having a gas inlet pipe 11 entering at the top and an air inlet pipe 12 entering at one end. The gas pipe 11 is connected by suitable piping to the flexible hose 13 which in turn is connected to a suitable gas supply. The air pipe 12 is likewise connected to a flexible hose 14 which is connected to any suitable supply of air under pressure. Pipe 12 terminates inside of the T 10 in the tapered

atomizing-nozzle 15. To the other end of the T 10 is connected an enlarged mixing tube 16 having attached to its end at a slight angle the burner-tip 17. This burner-tip is shown in section in Fig. 3. It will be seen that within this tip is mounted a cylindrical casting of correct size as indicated by 19 to leave a space 20 between its outer surface and the inner wall of the tip. At the extreme outer end the casting is provided with an outwardly extending circular flange 23 of a diameter slightly smaller than the inside diameter of the tip, leaving a circular space or crack 24 between such flange and the inner wall of the tip. Four holes are drilled through the casting. These holes are indicated by 26. The casting is held in place by a set screw 29. The torch is operated by gas and air of proper proportions to form an inflammable mixture which will burn at the end of the burner-tip. The purpose of the casting inside the tip is as follows. As the torch is in use the space 20 will be filled with inflammable mixture entering through the holes 26. If the gas is inadvertently turned off causing the torch to go out, or if the torch blows out, or goes out from any other cause, the mixture in the space 20 will burn very slowly at the crack 24 until it is entirely used up. Since this crack is very small, this burning will continue for some time after the torch has gone out. Such burning serves therefore in the nature of a pilot-light by which the torch may again be relighted by merely turning on the proper supply of gas and air.

In the practice of my invention I provide a plate or die 30 formed of cast iron or any other suitable material of appropriate dimensions, having formed in its upper surface grooves or sunken portions delineating the letter or figure which it is desired to form in the glass. As here shown, the die 30 or plate 30 is formed with a letter "E." The die or plate 30 is placed upon a suitable table or other support 31. I then provide a sheet of glass 32 of appropriate dimensions to cover the die. I then place the sheet of glass on the die so that the sunken portions are covered. I then light the torch A and direct the flame thereof indicated by 35 downwardly onto the sheet of glass. The heat softens the glass until it is sufficiently yielding so that the pressure caused by the blast will force it completely down into

the depressions in the dies causing it to conform to the surface of such depressions. Gravity assists the process. As shown in Fig. 10 the portion of the glass sheet 32 <sup>5</sup> directly under the flame 35 has already been softened and forced down into the depression in the die. The flame is moved over the die until the sheet of glass has been softened and pressed down into the mold at all points.

10 When this process has been completed the glass will appear as shown in Fig. 8. The glass is then allowed to cool until it is hard, whereupon the plate 30 may be removed and turned over as shown in Fig. 9, so that the <sup>15</sup> letter that was formed will appear in relief as indicated by 50.

In carrying out my improved process, the blow-torch flame should not be applied directly to a cold sheet of glass since this <sup>20</sup> might cause such a sudden change of temperature as to crack the glass. It will be found desirable to preheat the glass gradually to a certain extent first before placing it on the die and before applying the blow-torch <sup>25</sup> flame thereto. It will also be found desirable to heat the die to a certain extent separately before laying the sheet of glass upon it, so that there will be no chilling effect upon the glass which might crack it. In other <sup>30</sup> words, proper precaution should be taken, as suggested above, or in any other manner to prevent any damage to the glass. Likewise, after the completion of the process the glass should be properly annealed.

35 Although the present invention has been described by describing in detail one particular method of carrying it out, it is not intended that these details shall be regarded as limitations upon the scope of the invention except in so far as included in the accompanying claims.

I claim:

1. The method of producing a raised character in a sheet of glass, which includes the <sup>40</sup> providing of a die having on its surface a

depression corresponding to the character to be formed, the placing of a sheet of glass on the die to cover such depression, and the applying of a flame from a blow-torch downwardly and directly on to the portion <sup>45</sup> of said glass over such depression and with such pressure as to heat, soften, and force said glass mainly thereby into such depression.

2. The method of producing a raised <sup>50</sup> character in a sheet of glass, which includes the applying of a flame from a blow-torch downwardly and directly on to said sheet of glass to heat, soften and force said glass mainly thereby into an intaglio die placed <sup>55</sup> beneath said sheet of glass, said die having on its surface a depression corresponding to the character to be formed.

3. The method of producing a raised character in a sheet of glass, which includes the <sup>60</sup> supporting of the sheet in such a manner as to leave unsupported portions thereof corresponding to the character to be formed, and the applying of a flame from a blow-torch downwardly and directly on to the unsupported <sup>65</sup> portions of said glass to heat, soften and depress said portions mainly thereby.

4. The method of producing a raised character in a sheet of glass, which includes the <sup>70</sup> providing of a die having on its surface a depression corresponding to the character to be formed, the placing of a sheet of glass on the die to cover such depression, and the applying of a flame from an adjustable <sup>75</sup> blow-torch downwardly and directly on to the portion of said glass over such depression and with such pressure as to heat, soften, and force said glass mainly thereby into such depression.

In witness whereof I have hereunto set my hand and seal this 28th day of March, 1921.

EUGENE C. GMELIN. [L.S.]